

1,364,620.

J. R. DRANEY,

PAVEMENT,

APPLICATION FILED JULY 14, 1916.

Patented Jan. 4, 1921.

Fig. 1.



Fig. 2.



Inventor

Joseph R. Draney,

WITNESS:-

Chas. L. Griesbauer

By Cushman, Bryant & Darby  
Attorneys

# UNITED STATES PATENT OFFICE.

JOSEPH R. DRANEY, OF RIDGEWOOD, NEW JERSEY, ASSIGNEE, BY MESNE ASSIGNMENTS, TO BITOSLAG PAVING COMPANY, OF NEW YORK, N. Y., A CORPORATION OF DELAWARE.

## PAVEMENT.

1,364,620.

Specification of Letters Patent. Patented Jan. 4, 1921.

Application filed July 14, 1916. Serial No. 109,262.

*To all whom it may concern:*

Be it known that I, JOSEPH R. DRANEY, a citizen of the United States, residing at Ridgewood, in the county of Bergen and 5 State of New Jersey, have invented new and useful Improvements in Pavements, of which the following is a specification.

The present invention relates to pavements, and has to do more particularly with 10 pavement foundations, which foundations are laid upon the prepared ground, so that a bed of sufficient rigidity to withstand traffic strains, temperature changes, and the like is secured, over which foundation any 15 suitable or desired wearing surface may be placed.

In the building of roadway foundations it has been customary, and in fact almost the universal practice, to make that foundation 20 of broken stone, which is sized and compacted so as to give a rigid structure, and it has further been the practice to bind by cement such broken stone, so that a foundation of great rigidity, over which a suitable 25 wearing surface, usually bituminous, may be placed, is provided.

A pavement so constructed while having the advantage of furnishing a rigid foundation, presents certain disadvantages from a 30 practical standpoint, one of which is that it is not entirely waterproof, and when the wearing surface is destroyed is subject to the attacks of moisture, which results in its rapid deterioration, and compels the utilization 35 of a water repellent wearing surface so as to prevent moisture from reaching and attacking the foundation.

Again there is not such cohesion of the 40 wearing surface and the foundation as is desirable, owing to the structural differences between foundation and wearing surface, and the organic differences in the materials used, and, furthermore, such a foundation has not the resiliency which is desirable. 45 Furthermore the matter of laying such foundations requires a large amount of preliminary work before the wearing surface can

be applied, and in building both the stone and the stone and cement foundations considerable time is consumed, both in the application of the stone and cement material to the prepared ground, and the setting of this material prior to the application of the wearing surface.

My present invention is designed to, and 55 does, in fact, overcome the objections noted in connection with the class of pavement just discussed, and it contemplates the use as a foundation element of a particular kind of asphalt combined with a suitable mineral 60 aggregate, and so laid as that the work of laying the foundation may be expeditiously proceeded with, its union with the wearing surface will be much better, and its coefficient of resiliency will be higher than that 65 of the ordinary foundation, although a rigidity sufficient to meet traffic requirements is secured.

I accomplish these objects by using a mixture of "blown" or oxidized asphalt with a 70 suitable mineral aggregate graded to such mesh as will give a readily workable and coherent mixture, and I have found that good results are obtainable from the use of coarse sand, such as is available in many localities. 75

Asphalt produced by oxidization from heavy asphaltic base petroleums is very economical, so that it may be advantageously used for foundations, and, furthermore, and what is material in the formation of roadway foundations, has a quality of rigidity 80 which is higher than that of the asphalt produced from petroleum bases by the ordinary distillation method.

While the cementing qualities of such oxidized asphalt are less than the usual distilled asphalt, yet it is not so easily affected by the change of temperature, and is less yielding, so that when combined with a mineral aggregate, which is preferably coarse 85 in comparison with the finer aggregate for surfacing mixtures, a base or foundation is secured which is sufficiently rigid to stand up 90 under traffic without danger of crawling or

disintegrating, and yet which has a certain desirable resiliency not found in the cement and rock bases commonly in use.

Blown asphalt has several advantages over the binders now commonly in use in making foundations. It is less fluid than distilled asphalt and, therefore, is a more stable constituent and one which will resist any tendency of the foundation to shift under traffic 5 stresses. It is less susceptible to temperature and will not soften at high temperatures which would tend to cause flowing of distilled asphalt; though its quality is such that low temperatures do not cause any undue or deleterious brittleness. It gives up its oil content very slowly, so that its life is much prolonged and its resiliency maintained over a considerably longer period than the ordinary distilled asphalt.

10 These qualities render it peculiarly well-fitted for foundations, where resiliency, stability, immunity from temperature changes, and repellence of the attacks of moisture are highly essential; and, what is also important 15 it gives the foundation an affinity for wearing surfaces which is desirable and tends to a homogeneity of the road structure which is much to be desired.

In my experiments I have found that an oxidized asphalt from various petroleums may be utilized, but that produced from Mexican petroleum is preferable, as the resulting product has proved to be superior in some respects to the products from other petroleums.

While this foundation of mineral aggregate and oxidized asphalt may be laid in various ways, I have found that the method of depositing it in relatively thin layers or plies is advantageous, for the reason that if the deposit is too thick it is not easily handled, and the compression desired is difficult to obtain. The number of layers is immaterial, and will, of course, depend upon the traffic load which the road is designed to carry, but regardless of the number of layers of oxidized asphalt and mineral aggregate which are specified, the deposit of each layer should be a separate operation, and the layers 40 may, of course, differ in thickness if desired, and in such case the heaviest layer would preferably be the bottom layer. The several layers should preferably "set" or "cure" prior to the application of the succeeding 45 layer, but a mixture of this type after compression by a roller, or other means, sets very quickly, so that the work of building up a foundation can proceed expeditiously, and the delay incident to curing or setting 50 cement foundations is done away with, foundations of this type requiring a considerable period of curing before it is possible to apply the wearing surface.

In order that the invention may be clear

to those skilled in the art, I have illustrated 55 in the accompanying drawing conventionally my invention.

In said drawing:

Figure 1 is a cross-sectional view of a portion of a roadway showing conventionally 70 my construction and method of laying roadway.

Fig. 2 is a view similar to Fig. 1 showing a single foundation layer as distinguished from the plurality of foundation layers 75 shown in Fig. 2.

Referring to the drawings by numerals, like numbers indicating like parts in the several views, 10 indicates the sub-base or earth upon which the roadway is laid.

The foundation layers are indicated by numerals 11, these being deposited as stated upon the sub-base.

The top or wearing surface is indicated by the numeral 12, which top or wearing surface may, of course, be of any suitable adherent material.

In the form shown in Fig. 2, I have illustrated the use of one foundation layer 11 as distinguished from the use of a plurality of 90 layers.

With the asphaltic foundation prepared in accordance with my invention may be used any suitable wearing surface, and a very desirable union between the foundation and 95 the wearing surface will be secured, particularly if the not uncommon asphaltic wearing surface made up of asphalt and a fine mineral aggregate be used, so that a better balance is brought about between the foundation and the wearing surface, and the liability of separation and crawling of one relative to the other is much reduced. Furthermore this foundation while rigid enough to withstand traffic strains has an element of 100 resiliency not found in the cementitious foundations, giving a more yielding base, and one which will relieve to a considerable extent the tendency of the wearing surface to disintegrate or move under traffic.

I claim:-

1. A pavement comprising a foundation formed of a mixture of oxidized asphalt and mineral aggregate, and an adherent wearing surface applied to said foundation.

2. A pavement comprising a foundation formed of a mixture of oxidized asphalt and mineral aggregate, and an adherent wearing surface of non-oxidized asphalt and mineral aggregate to said foundation.

3. The herein described composition for the foundation of a pavement comprising a mixture of oxidized asphalt and mineral aggregate.

4. The herein described composition for a 125 pavement foundation comprising a mixture of oxidized asphalt from Mexican petroleum and mineral aggregate.

5. The herein described method of forming roadways which consists in laying a foundation comprising a plurality of superposed, independently applied layers of a mixture of oxidized asphalt and mineral aggregate, and applying to such foundation an adherent wearing surface.
6. The herein described method of forming roadways which consists in laying a foundation layer of oxidized asphalt and a mineral aggregate upon a suitable bed, allowing such layer to cure or set to an appreciable degree, applying successive layers
- 10
- to said first named layer and allowing each successive layer to cure before applying a succeeding layer, until the desired thickness of foundation is secured, and applying to such foundation an adherent wearing surface.
- In testimony whereof I have hereunto set 20 my hand in presence of two subscribing witnesses.

JOSEPH R. DRANEY.

Witnesses:

M. F. ODUL,  
F. ODONE.